

Dec. 16, 1930.

C. H. SEYMOUR

1,785,502

METAL BEARING MEMBER AND PROCESS OF TREATING SAME

Filed Aug. 26, 1927

*Fig 1*



*Fig 2*



Charles H. Seymour, INVENTOR  
BY  
Warren W. House, ATTORNEY

## UNITED STATES PATENT OFFICE

CHARLES H. SEYMOUR, OF KANSAS CITY, MISSOURI

## METAL BEARING MEMBER AND PROCESS OF TREATING SAME

Application filed August 26, 1927. Serial No. 215,625.

My invention relates to improvements in metal bearing members and processes of treating same.

One of the objects of my invention is to provide a novel process for treating metals, used for various purposes, such as in bearings, and lead plates of storage batteries, in a novel manner by which the heating thereof by use will be eliminated or greatly reduced, as compared with metal not so treated.

A further object of my invention is to provide a novel process of treating alloys and non-hardening metals so as to reduce the liability of their becoming highly heated in use.

Still another object of my invention is the provision of a novel bearing member which will not become heated when subjected to conditions which cause heating of the usual bearing member.

The novel features of my invention are hereinafter fully described and claimed.

In the accompanying drawing,

Fig. 1 is an elevation of a bearing of the usual type employed to support rotating shafts.

Fig. 2 is a plan view of the same.

Similar reference characters designate similar parts in the different views.

In carrying my invention into effect, the metal to be treated is cooled in an oleoresinous substance, such as turpentine, while heated to a temperature above the boiling point of the oleoresinous material, and, preferably between such point and the point at which the metal treated fuses.

In treating a bearing, such as is shown in the drawing, the upper and lower members, 1 and 2 respectively, thereof are first heated to a temperature as high as the boiling point of the oleoresinous material, such as turpentine.

The temperature employed may be any between the boiling point of the immersing material and the fusing point, or slightly below, the fusing point of the metal of which the bearing members are composed. The heating is not brought at a higher temperature, as such would deface or ruin the members for the purpose for which they are provided.

After the bearing members have been immersed in the turpentine until cooled, they may be immediately used in the usual manner, and bearings so treated will not become heated to anything like bearings not so treated, which are subjected to like conditions of use.

Lead plates used in storage batteries, after being treated in the manner described, will not become heated when subjected to use corresponding to such that, with plates, not similarly heated, will cause the latter to become heated.

Many bearings are manufactured which are composed of an alloy consisting of copper, tin, lead, zinc, with, sometimes a small amount of antimony. Bearings of the usual commercial kind so made and subjected to the treatment of my improved process will be practically immune from heating under conditions of use that will soon cause heating of bearings made of the same alloy, but not so treated.

Most any soft, nonhardening metal or alloy, in fact all such metals or alloys that I have treated by my improved process become practically immune to heating from friction against revolving parts, or from eddy currents, such as are frequently formed in soft iron cores.

The usual babbitt, bronze or brass bearing members, when subjected to my improved treatment, as hereinbefore described, become practically immune to heating by use that would cause them to become highly heated, if they were not so treated.

Various modifications of my invention, within the scope of the appended claims may be made without departing from the spirit of my invention.

What I claim is:—

1. The process consisting in cooling in contact with an oleoresinous material a bearing member of the kind described comprising soft non-hardening metal heated to a temperature between the boiling point of said material and the fusing point of the metal.

2. The process consisting in cooling in contact with an oleoresinous material a bearing member of the kind described comprising

ing a non-hardening alloy heated to a temperature between the boiling point of said material and the fusing point of the alloy.

3. The process consisting in cooling in contact with turpentine a bearing member of the kind described comprising soft non-hardening metal heated to a temperature between the boiling point of turpentine and the fusing point of the metal.

10 4. The process consisting in cooling in contact with turpentine a bearing member of the kind described comprising, a non-hardening alloy heated to a temperature between the boiling point of the turpentine and the fusing point of the alloy.

15 5. The process consisting in cooling in contact with an oleoresinous material, a bearing member of the kind described comprising a relatively soft non-hardening alloy containing 20 copper heated to a temperature between the boiling point of the material and the fusing point of the alloy.

25 6. The process consisting in cooling in contact with an oleoresinous material, a bearing member of the kind described comprising a relatively soft non-hardening alloy containing tin heated to a temperature between the boiling point of the material and the fusing point of the alloy.

30 7. The process consisting in cooling in contact with an oleoresinous material a bearing member of the kind described comprising a relatively soft non-hardening metal heated to a temperature as high as the boiling point of said material.

35 8. The process consisting in cooling in contact with an oleoresinous material a bearing member of the kind described comprising a non-hardening alloy heated to a temperature as high as the boiling point of said material.

40 9. A bearing member of the kind described composed of a relatively soft non-hardening metal which has been cooled in contact with an oleoresinous material while heated to a temperature between the boiling point of the material and the fusing point of the metal.

45 10. A bearing member of the kind described composed of a relatively soft non-hardening alloy which has been cooled in contact with an oleoresinous material while heated to a temperature between the boiling point of the material and the fusing point of the alloy.

50 11. A bearing member of the kind described composed of a relatively soft non-hardening alloy containing copper and which has been cooled in contact with an oleoresinous material while heated to a temperature between the boiling point of said material 55 and the fusing point of the alloy.

55 12. A bearing member of the kind described composed of a relatively soft non-hardening alloy containing tin and which has been cooled in contact with an oleoresinous material while heated to a temperature be- 60

65 tween the boiling point of said material and the fusing point of the alloy.

70 13. The process consisting in cooling in contact with an oleoresinous material a bronze bearing member of the kind described heated to a temperature between the boiling point of said material and the fusing point of said bronze.

75 14. The process consisting in cooling in contact with turpentine a bronze bearing member of the kind described heated to a temperature between the boiling point of said turpentine and the fusing point of said bronze.

80 15. A bronze bearing member of the kind described which has been cooled in contact with an oleoresinous material while heated to a temperature between the boiling point of said material and the fusing point of said bronze.

85 16. A bronze bearing member of the kind described which has been cooled in contact with turpentine while heated to a temperature between the boiling point of said turpentine and the fusing point of said bronze.

90 In testimony whereof I have signed my name to this specification.

CHARLES H. SEYMOUR.

89

95

100

105

110

115

120

125

130

135

140